

## UNITED STATES PATENT OFFICE

2,414,839

## LIGHT SENSITIZED LEAD PRINTING COMPOUNDS AND PROCESS OF REPRODUCTION

André Schoen, Easton, Pa., assignor to General Aniline &amp; Film Corporation, New York, N. Y., a corporation of Delaware

No Drawing. Application January 31, 1945,  
Serial No. 575,557

15 Claims. (Cl. 95—6)

1

The present invention relates to light sensitive printing papers and the like containing lead compounds and to the process of image development thereof. It relates also to the super-sensitization of such compounds to increase the speed or sensitivity thereof to light.

Heretofore, it has been proposed to employ the light sensitive compounds of lead in photographic processes, and develop the latent image by a physical developer, but such processes have not attained any commercial importance, possibly due to the difficulties in development thereof and the long exposure time required for formation of the latent image.

It is an object of the present invention to provide a process for chemically developing light sensitive lead compositions.

Another object of the present invention is to super-sensitize, that is, increase the sensitivity to light of, light sensitive lead compounds.

A further object is the provision of a photographic process employing a suitable base carrying a light sensitive lead compound.

According to one feature of the present invention the latent image on a base carrying a light sensitive lead compound which has been exposed to light under a pattern or the like to be reproduced, is developed by treatment with a strong reducing agent, resulting in a print or photograph in black and white. The invention may be carried out in practice by coating any suitable base with a light sensitive lead compound, and after drying, the base is exposed to a suitable source of light under a suitable negative carrying the design to be reproduced, then the base is developed in a solution having a strong reducing action, and is washed and dried. By the term "strong reducing agent" I mean an agent with sufficient reducing potential to bleach or discharge azo dyes, for example, Beta Naphthol Orange (C. I. 151).

In accordance with another feature of the invention, the sensitivity to light of lead compounds supported on a suitable base is enhanced by treatment with a substance containing a thiocarbonyl radical, especially an aminothiocarbonyl radical, such as a thiocarbamido group. Examples of such substances are, sodium sulfoxylate formaldehyde, sulfinoformamidine or allylthiourea. Compositions so treated after exposure to light, are preferably developed with a strong reducing agent in solution as above described.

Preferably the light sensitive lead compounds which are water insoluble are precipitated on the support, such as a paper sheet, plate or the like, by a base exchange reaction in aqueous solution,

although if desired, a gelatin solution or emulsion of the light sensitive lead compounds may be applied. The lead compounds may be treated with the supersensitizing material before, at the same time or after being applied to the base, carrier or support as desired. Preferably the base is first treated with a soluble lead compound and then is treated in the dark with a soluble base exchange compound to precipitate on the base the insoluble light sensitive compound. Thus, the supersensitizing compound may be present in one of the base exchange solutions, or may be applied after precipitation of the insoluble light sensitive lead compound.

Light sensitive sheets, plates or the like thus prepared preferably are employed in the printing through process wherein light is transmitted from a suitable source through the negative to the sensitized lead compound coated sheet for the required time to develop a latent image, which is then developed by solutions of strong reducing agents. Such strong developer solutions may be used to develop sheets carrying light sensitive lead compounds with or without treatment with the supersensitizer herein described, and no fixing of the developed image is required. However, the stability of the developed image to moisture may be improved by treating the developed base with a moisture stabilizer such as, for example, a solution of a soluble ionized chloride, such as sodium chloride, or cadmium chloride, or ammonia, or potassium dichromate or the like. I believe the moisture stabilizers provide a protecting layer of an insoluble lead compound, but do not wish to be limited to this theory in claiming my invention.

The lead image may be toned by any of the toners free from sulfides employed for silver images, for example, by treatment with a solution containing potassium ferricyanide, ferric ammonium citrate and acetic acid, which changes the image to blue and renders the image more stable. Preferably, such toners free from noble metals are employed.

As suitable light sensitive lead compounds there may be employed, for example, lead iodide, lead azide or lead bromide, which exhibit decreasing sensitivity to light in the order named.

In particular I have found that in the example of a base coated with lead azide and supersensitized with sodium sulfoxylate formaldehyde, by a sufficiently long exposure to light rich in ultra violet rays a black print may be obtained directly that is, without development with a reducing agent, although in general it is preferred to carry

out the exposure for a shorter time and develop the latent image with a strong reducing agent. As examples of suitable strong reducing agents having a reducing potential sufficient to bleach or discharge azo dyes, may be mentioned sodium hydrosulfite, sodium stannite, sulfinoformamide ( $\text{HSO}_2\text{CNH}_2:\text{NH}$ ), titanous chloride, titanous sulfate or the like.

The invention will be described in further detail in connection with the following examples which are given to illustrate the invention.

*Example I*

A sensitized paper is prepared by treating a paper base with a solution of 20 g. lead acetate in 100 cc. water, drying, then treating the paper in the dark with a solution of 20 g. potassium iodide in 100 cc. water, drying, and then treating the paper in the dark with a solution of 10 g. sodium sulfoxylate formaldehyde in 100 cc. water and drying. The sensitized paper is exposed under a negative in a printing frame for about one half second to the light from a photoflood lamp located 16 inches from the printing frame, and the exposed paper is then developed in a solution of 20 g. anhydrous sodium carbonate and 8 g. sodium hydrosulfite in a liter of water for about one minute at 45° C. The developed positive is then treated for about two minutes in a solution of sodium chloride of about five to ten percent strength and then dried. There results a positive black and white print.

*Example II*

A paper base coated with lead azide is prepared by first treating the paper with a solution of 20 g. lead acetate in 100 cc. water, drying, then treating it in the dark with a solution of 15 g. sodium azide in 100 cc. water and drying. The light sensitive paper is exposed to a suitable source of light under a negative to form a latent image which is then developed as described in Example I. The developed positive is then treated for about two minutes in a solution of sodium chloride of about five to ten percent strength, and then dried. There results a positive black and white print.

I claim:

1. The process which comprises exposing to light under a pattern to be reproduced a light-sensitive layer on a suitable support comprising a light-sensitive lead compound and developing the thus formed latent image in a solution of a strong reducing agent selected from the group consisting of sodium hydrosulfite, sodium stannite, titanous chloride and titanous sulfate.
2. The process which comprises exposing to light under a pattern to be reproduced a light-sensitive layer on a suitable support comprising a light-sensitive lead compound and a supersensitizing agent selected from the group consisting of sodium sulfoxylate formaldehyde, sulfinoformamidine, and allylthiourea and developing the latent image thus formed in a solution of a strong reducing agent selected from the group consisting of sodium hydrosulfite, sodium stannite, titanous chloride and titanous sulfate.

3. The process which comprises exposing to light under a pattern to be reproduced a light-sensitive layer on a suitable support comprising a light-sensitive lead compound and developing the thus formed latent image in a solution of an alkali metal hydrosulfite.

4. The process which comprises exposing to light under a pattern to be reproduced a light-sensitive layer on a suitable support comprising a light-sensitive lead compound, developing the thus formed latent image in a solution of an alkali metal hydrosulfite and treating the developed image with a soluble inorganic chloride moisture stabilizer.

5. The process which comprises exposing to light under a pattern to be reproduced a light-sensitive layer comprising lead iodide on a suitable support and developing the latent image thus formed in a solution of sodium hydrosulfite.

6. The process which comprises exposing to light under a pattern to be reproduced a light-sensitive layer on a suitable support comprising lead iodide and sodium sulfoxylate formaldehyde and developing the latent image thus formed in a solution of sodium hydrosulfite.

7. The process which comprises exposing to light under a pattern to be reproduced a light-sensitive layer comprising lead bromide on a suitable support and developing the latent image thus produced in a solution of sodium hydrosulfite.

8. The process which comprises exposing to light under a pattern to be reproduced a light-sensitive layer on a suitable support comprising lead bromide and sodium sulfoxylate formaldehyde and developing the latent image thus formed in a solution of sodium hydrosulfite.

9. The process which comprises exposing to light under a pattern to be reproduced a light-sensitive layer comprising lead azide on a suitable support and developing the latent image thus produced in a solution of sodium hydrosulfite.

10. The process which comprises exposing to light under a pattern to be reproduced a light-sensitive layer on a suitable support comprising lead azide and sodium sulfoxylate formaldehyde and developing the latent image thus produced in a solution of sodium hydrosulfite.

11. A light-sensitive article comprising a support carrying a light-sensitive lead compound and a supersensitizing agent selected from the group consisting of sodium sulfoxylate formaldehyde, sulfinoformamidine and allylthiourea.

12. A light sensitive article comprising a support carrying a light sensitive lead compound supersensitized with sodium sulfoxylate formaldehyde.

13. A light sensitive article comprising a support carrying lead iodide supersensitized with sodium sulfoxylate formaldehyde.

14. A light sensitive article comprising a support carrying lead bromide supersensitized with sodium sulfoxylate formaldehyde.

15. A light sensitive article comprising a support carrying lead azide supersensitized with sodium sulfoxylate formaldehyde.

ANDRÉ SCHOEN.